

Patented Nov. 11, 1930

1,780,943

# UNITED STATES PATENT OFFICE

GEORGE A. RICHTER AND MILTON O. SCHUR, OF BERLIN, NEW HAMPSHIRE, ASSIGNEES  
TO BROWN COMPANY, OF BERLIN, NEW HAMPSHIRE, A CORPORATION OF MAINE

## FIBER LIBERATING AND BLEACHING PROCESS

No Drawing.

Application filed April 19, 1927. Serial No. 184,879.

This invention relates to the liberation and bleaching of cellulose fiber, and has for its object the production of fiber suitable for manufacture into papers of high pop test, 5 whiteness, and color stability.

After cellulose fiber is liberated from raw cellulosic material, such as wood chips, it is washed, screened, and, if intended for manufacture into writing papers or the like, finally 10 bleached. During such bleaching, oxycelluloses are produced in the fiber by degradation of its cellulose content,—increase in whiteness being accompanied by a lowering of the alpha cellulose content of the fiber 15 and injury to its paper-making characteristics. This is especially true in the case of a strong sulphite fiber produced by under-digesting in a liquor of high combined SO<sub>2</sub> content,—for instance, in a liquor having a combined SO<sub>2</sub> content considerably above that of 20 the usual calcium bisulphite liquor. The resulting fiber, while of high strength, is nevertheless difficultly bleachable, and if it be attempted to bleach such fiber to whiteness, its 25 papermaking qualities are severely injured.

In accordance with the process of our invention, the bleaching of fiber, such for instance as that liberated in liquor of high combined SO<sub>2</sub> content, is effected in a manner to 30 preserve its papermaking characteristics. Such bleaching, we carry out in two separate steps, the first of which consists in treating the unbleached fiber with chlorine water of a strength insufficient to whiten it, for if the 35 fiber were so whitened, it would be injured in papermaking characteristics. The chlorine-treated fiber is then whitened in a distinctly alkaline bleach liquor, in which the fiber may 40 be brought to substantially ultimate whiteness without material degradation of its cellulose content or injury to its papermaking characteristics. Apparently the free alkali in the bleach liquor increases the selectivity 45 of oxidation upon the lignous and coloring

materials, which are more susceptible to oxidation than is the cellulose.

An example of procedure which may be followed in producing white fiber of high strength and stability may be substantially as follows. Chipped wood,—spruce, for example,—is digested under pressure at an elevated temperature in a sodium bisulphite liquor containing about 4% combined and 4% free SO<sub>2</sub>, until complete fiber liberation has been effected. Digestion in a liquor of such high combined SO<sub>2</sub> results in a rapid penetration of the combined SO<sub>2</sub> into the chips, and results in a complete fiber liberation in a much shorter time than when the usual calcium base sulphite liquor containing about 1% combined SO<sub>2</sub>, and which is of much lower penetrability, is employed. The resulting fiber yield is higher and the fiber is of considerably greater strength than in the case of the usual sulphite pulp. This is probably ascribable to the fact that the fibers are longer and contain a larger proportion of the pentosan and lignous content of the wood, as a result of lower hydrogen ion 50 concentration in the liquor and less hydrolysis of fiber. Thus, whereas the usual unbleached sulphite pulp contains about 96% cellulose, pulp produced in a liquor containing about 4% combined and 4% free SO<sub>2</sub> may 55 contain about 85% to 95% cellulose, depending upon the thoroughness of cook, and is high in pentosans and lignous matter. If such a normal or undercooked pulp were 60 bleached as ordinarily, to a color of, say, about 100, its papermaking characteristics would be severely injured. In accordance 65 with our process, such pulp is first treated at a stock density of about 10% with chlorine water containing about 1.5% to 70 4% chlorine, based on dry fiber weight. The treatment may be carried out at about room temperature for about one-half hour or so, as the chlorine is rapidly 75 consumed by reaction upon lignous and other 80 85 90 95 98

coloring matter, removing or rendering such matter more susceptible to subsequent oxidation. Such treatment does not whiten the pulp, but tends to deepen its color to a distinct yellow or light orange. The treated pulp is washed and then bleached at a stock density of about 10% in a solution containing about 5% to 10% sodium or calcium hypochlorite and about 1/2% to 2% caustic soda, based on dry fiber. Bleaching may be carried out at about room, or at a temperature of 100 to 110° F., until the fiber is brought to substantially ultimate whiteness. Under such conditions, a whitening of the fiber is effected without injury to its papermaking characteristics or material degradation or the cellulose into oxycelluloses. Apparently, the free alkali not only tends to increase the selectivity of oxidation upon the ligneous matter, but also to dissolve out the ligneous reaction products of the chlorine treatment. The bleached pulp is washed and treated with an anti-chlor, e. g., sodium bisulphite, to remove residual chlorine and to neutralize it.

The bleached pulp has a high pop test and yields hard, ratty papers, so that it is particularly suitable for the manufacture of "glassine" papers and bond papers of high color, stability, and strength. Thus, papers formed from pulp liberated and bleached as hereinbefore described have a pop test of about 140 to 160, as compared with a pop test of about 115 to 125 of the usual sulphite pulp papers.

As hereinbefore stated, one of the advantages of our process is that wood pulp produced by digestion in a liquor having a high combined  $\text{SO}_2$  content may be whitened without materially injuring its papermaking characteristics. Such a process is economically advantageous, as a high yield of pulp is produced by digestion, which, in turn, is reflected in a higher yield of bleached pulp, such latter yield amounting to about 50%, based on wood, as compared with a yield of about 45% for the usual sulphite pulp. The bleached pulp has a high pop strength, and at the same time a tear resistance comparable to the usual sulphite pulp, and although of high color, possesses remarkable color stability and is low in copper number.

While we have described a specific example of procedure wherein pulp is liberated by digesting wood chips in a cooking liquor having a combined and free  $\text{SO}_2$  content of about 4% each, it should be understood that pulp liberated in other liquors, for instance, in the usual calcium bisulphite liquor or in sodium bisulphite or in mixed sodium bisulphite and calcium bisulphite liquors containing 2% combined and 5% free  $\text{SO}_2$ , or other proportions of combined and free, may be advantageously bleached as hereinbefore described.

Where liquors containing high combined  $\text{SO}_2$  contents are employed, the chips are prefer-

ably undercooked to produce hard, strong pulps, as our bleaching treatment is applicable to greatest advantage in such case.

The bleaching process herein described may be applied successfully to unbleached pulps other than sulphite, such for instance as well-cooked soda or kraft pulps, particularly when such latter pulps are liberated from such wood as birch, beech, maple, and poplar. It finds great utility, however, in the bleaching of hard, strong sulphite pulps to produce a high yield of strong, white fiber of high stability, as indicated by the specific example herein given.

Having thus described certain examples of procedures, it should be understood that these procedures might be deviated from without departing from the spirit or scope of invention as defined by the appended claims.

What we claim is:

1. A process which comprises treating unbleached pulp with chlorine water, and then bleaching such pulp in a bleach liquor maintained distinctly alkaline throughout such bleaching and containing sufficient bleach to whiten such pulp. 90

2. A process which comprises digesting wood chips in a sulphite liquor having a combined  $\text{SO}_2$  content considerably above that of the usual calcium bisulphite liquor, treating the resulting pulp with chlorine water, and bleaching the treated pulp in a distinctly alkaline bleach liquor containing sufficient bleach to whiten such pulp. 95

3. A process which comprises digesting wood chips in a sulphite liquor having a combined  $\text{SO}_2$  content considerably above that of the usual calcium bisulphite liquor and a free  $\text{SO}_2$  content about equal to its combined  $\text{SO}_2$  content, treating the resulting pulp with chlorine water but insufficiently to whiten it, and bleaching such pulp in a distinctly alkaline bleach liquor containing sufficient bleach to whiten such pulp. 100

4. A process which comprises digesting wood chips in a sodium bisulphite liquor having a combined and free  $\text{SO}_2$  content of about 4% each, treating the resulting pulp with chlorine water but insufficiently to whiten it, and bleaching such pulp in a distinctly alkaline liquor containing sufficient bleach to whiten such pulp. 115

5. A process which comprises undercooking wood chips in a sulphite liquor having a combined  $\text{SO}_2$  content considerably above that of the usual calcium bisulphite liquor, treating the resulting pulp with chlorine water of a strength which results in a deepening of the color of such pulp, and bleaching the treated pulp in a distinctly alkaline bleach liquor containing sufficient bleach to whiten such pulp. 120

6. A process which comprises digesting wood chips in a sodium bisulphite liquor hav-

70

75

80

85

90

95

100

105

110

115

120

125

130

ing a combined and free SO<sub>2</sub> content of about 4% each, treating the resulting pulp with chlorine water but insufficiently to whiten it, and bleaching such pulp in a hypochlorite bleach liquor maintained distinctly alkaline with caustic soda throughout such bleaching and containing sufficient bleach to whiten such pulp.

5 In testimony whereof we have affixed our signatures.

10 GEORGE A. RICHTER  
MILTON O. SCHUR.

15

20

25

30

35

40

45

50

55